

## UNITED STATES PATENT OFFICE

2,579,890

## NONCLOGGING DISTILLATE FUEL OIL

Calmy Wies, New York, N. Y., and John B. R. Caron, North Plainfield, and Everett B. Glendenning, Cranford, N. J., assignors to Shell Development Company, San Francisco, Calif., a corporation of Delaware

No Drawing. Application July 3, 1948,  
Serial No. 37,084

13 Claims. (Cl. 44—70)

**1** This invention pertains to improved hydrocarbon fuels, and more particularly to fuel oil compositions capable of preventing or inhibiting the sludging and/or clogging tendencies generally exhibited by hydrocarbon fuels, such as those utilized in burner systems, tanks, diesel and combustion engines, and various other industrial and domestic equipment. In addition, this invention relates to fuel compositions capable of removing preformed deleterious matter from filters, screens, and the like, caused by deterioration and/or the presence of foreign bodies e. g. water in fuel oils.

Hydrocarbons, such as distillate fuels, for example, those having a normal distillation range of from about 300° F. to 750° F. and particularly those fuels having a distillation range of from about 340° F. to about 640° F., generally have a marked tendency to deteriorate under oxidizing conditions, and to form sludge. Also, the presence of impurities in such fuels, such as the presence of moisture, dispersed water, organic and/or inorganic foreign matter, and the like, cause the formation of insoluble products, which tend to settle out and adhere to surfaces with which they come in contact, thereby in turn, causing clogging or plugging of filters, strainers, screens, conduit lines, and the like, of the equipment in which they are used. This necessitates frequent cleaning and even replacement of parts, thereby markedly decreasing the performance efficiency of various equipment which utilizes such fuel oils.

The problem of screen clogging is common, particularly in domestic fuel oil systems employing distillate fuel oils produced by distilling or cracking of petroleum which fuels are characterized by their relatively low viscosity and other properties. Fuel oils of this type generally conform to the specifications set forth in Commercial Standards C. S. 12-40 for Nos. 1, 2, and 3, fuel oils. Petroleum distillates within the ranges specified and which generally do not exceed 750° F. and preferably are below 675° F. for use as diesel fuels are further examples of the type of oils which under conditions described have a tendency towards screen or filter clogging, particularly when they contain minor amounts of water dispersed therein.

Another place where screen clogging and plugging of conduit lines is encountered is in storage tanks for fuel oils, which tanks may be connected to the burner systems or engines, etc. The stored fuel generally comes in contact with air, moisture, water, etc., which causes formation and precipitation of sludge materials which in turn settle out and deposit on and clog the screens

or filters used for protecting the burners or engines which use such oils as the fuel.

It is an object of this invention to inhibit sludging tendencies of hydrocarbon fuel oils. It is another object of this invention to inhibit sludging and precipitation of contaminants in hydrocarbon distillate fuel oils, and particularly in cracked hydrocarbon fuels. It is still another object of this invention to provide distillate fuel oils and particularly fuel oils obtained during cracking of hydrocarbons, which fuels have excellent performance characteristics with respect to freedom from screen clogging, even after extensive storage under oxidizing conditions and in the presence of water. Still another object of this invention is to provide a distillate fuel oil composition which is effective in removing preformed sludge deposits formed in fuel oil systems. Still another object of this invention is to provide a particular type of distillate fuel oil compositions, and blends thereof, which are non-corrosive and stable, and which are effective for cleaning and sludge removing.

The above and other objects of this invention may be attained by dispersing or dissolving in a hydrocarbon distillate fuel oil (which normally have a tendency to cause clogging or plugging of screens, filters, conduit lines and the like) a minor amount, which amount, however, is sufficient to inhibit said tendencies, of a specific class of surface active agents such as the salts of a sulfo carboxylic acid ester, and derivatives thereof. If desired, a minor amount of a detergent and/or drying agent or solutizer may be added to the composition.

35 The hydrocarbon distillate fuel oils in which the active ingredient and/or ingredients of this invention are dispersed or dissolved may be treated or untreated cracked fuel oils, or mixtures of cracked fuels with straight run fuel oils, having components normally distilling at about 500° F. and having an end distillation point not exceeding 750° F. Generally such fuels of the type under discussion have a boiling range of from about 340° F. to about 700° F. and preferably have a boiling range of from about 400° F. to about 675° F.

Cracked fuels may be obtained by thermal or catalytic cracking of certain petroleum hydrocarbon feed stocks. Both the cracked fuels as well as blends of cracked and straight run fuels, may be acid and/or caustic treated to improve their stability. Specifically, hydrocarbon distillates which are utilized as bases in compositions of this invention are cracked gas oils, fuel oils, furnace oils, burner oils, diesel fuel oils, kerosene,

etc., and mixtures of said cracked fuels with the corresponding or like straight run hydrocarbon fractions, e. g. fuel oils, etc.

The properties of a caustic treated catalytically cracked light gas oil and a 50-50 blend of an untreated catalytically cracked light gas oil and a straight run acid treated gas oil which have a marked tendency towards clogging screens, etc. are given in the following table:

| Properties                                       | 50-50 Blend of Catalytically cracked light Gas Oil and Straight Run Light Gas Oil | Catalytically Cracked Light Gas Oil |
|--------------------------------------------------|-----------------------------------------------------------------------------------|-------------------------------------|
| Gravity, ° API                                   | 32.6                                                                              | 31.0                                |
| ASTM Dist (° F)                                  |                                                                                   |                                     |
| IBP                                              | 414                                                                               | 434                                 |
| EBP                                              | 664                                                                               | 620                                 |
| Sulfur Per Cent W.                               | 0.839                                                                             | 0.783                               |
| Conradson Carbon Residue (10% Btms) (Per Cent W) | 0.01                                                                              | 0.01                                |
| Pour Point, ° F                                  | 5                                                                                 | -5                                  |

The surface active agents which possess the unique property of inhibiting sludge formation or removing preformed deposits from surfaces thereby preventing clogging of systems utilizing fuels normally susceptible of causing such deterioration are salts of organic acidic compounds containing a sulfo radical or radicals represented specifically by the following class of compounds:

IA. Salts of sulfopolycarboxylic acid esters such as are fully and clearly described in U. S. Patents, 2,028,091 and 2,176,423, and which may be broadly defined as derivatives of esters of aliphatic dibasic acids having the formula



wherein R is an alkyl radical containing at least one sulfonic group and X is hydrogen or an alcohol or phenol radical not connected by a carbon to carbon bond with R, at least one X being such an alcohol or phenol radical.

These sulfocarboxylic acid esters may be in the form of salts of alkali, alkaline earth or heavy metals such as Na, K, Li, Ca, Ba, Sr, Mg, Zn, Al, Sn, Cd, Cr, Sn, Ni, Fe or in the form of salts with ammonium or other amine bases. Specific acids used to form these compounds may be sulfosuccinic, sulfoadic, sulfoglutamic, sulfosuberic, sulfomalic, sulfomalic and other sulfodicarboxylic acids. Examples of specific compounds are: dioctyl sodium sulfosuccinate, diamyl sodium sulfosuccinate, dicapryl sodium sulfosuccinate, difurfyl sodium sulfosuccinate, dioctyl sodium sulfoadic, dioctyl sodium sulfomalic, etc. The amount of salt used may vary from about 2% to 10% and preferably between about 4% and 8%.

IB. Salts of alkyl esters of monocarboxylic aromatic sulfonic acids having the general formula:



wherein Ar is an aryl nucleus derived from hydrocarbons such as benzene, naphthalene, diphenyl and the like; X is a substituent such as hydrogen, hydroxyl, hydrosulfide, halogen and the like; Y is an alkali, alkaline earth or heavy metal such as Na, K, Li, Ca, Ba, Sr, Mg, Zn, Al, Ca, Cd, Cr, Sn, Ni, Fe; n, m, and p, are whole

numbers which may be one or a greater number; and R is an alkyl radical having from 8 to 18 carbon atoms. Compounds within the scope of this formula are: octyl-o-sodium sulfobenzoate, dodecyl-o-sodium sulfobenzoate, tetradecyl-o-sodium sulfobenzoate, boralkyl-o-sodium sulfobenzoate, dodecyl-p-sodium sulfobenzoate, dodecyl-m-sodium sulfobenzoate, dodecyl sodium sulfo-phenylacetate, di-n-hexyl ester of sodium 4-sulfophthalic acid, di-n-hexyl ester of potassium sulfophthalic acid, etc.

IC. The salts of sulfuric acid derivatives of reaction products of an alcohol and a hydroxy substituted aromatic compound, e. g. alkali alkaline earth heavy metal and ammonium salts of sulfuric acid derivatives of isopropyl, normal butyl, isobutyl, normal amyl alcohols, and ortho and/or para hydroxy diphenyl, etc.

If desired, and under certain conditions of use, it is preferred to add detergents to compositions of this invention. The function of the detergent agents in compositions of this invention appear to act as peptizers, to aid in inhibiting or preventing the settling and adhering of impurities and sludge to surfaces, and to allow any impurities present or formed to pass through the screen or filter system.

Detergents which may be used are alkali, alkaline earth and heavy metals and organic nitrogen base salts of various organic acids. The acidic portion of such detergents may be naphthenic acids, petroleum sulfonic acids, aromatic and hydroxy aromatic carboxylic acids, aliphatic acids, said acids containing, if desired substituent groups, e. g. amino, hydroxide, mercapto, halogen and sulfur groups and the like. Also phenates, alcoholates, carbamates, thiocarbamates, xanthates, etc., may be used.

Particularly preferred class of detergents are the salts of alkyl substituted phenol sulfides, or its selenide and/or its telluride equivalents. These phenolic salts may be represented by the general formulas



wherein M is a metal; R and R' represent at least one alkyl radical attached to the aromatic ring Ar, the total number of carbon atoms in all of such radicals being at least 5; X is O and/or S; Q is S, Se or Te and n is an integer of from 1 to 4.

To form the salts of these phenolic compounds they may be treated with such metal compounds, as Li, Na, K, Cu, Hg, Fe, Mn, Mg, Ca, Ba, Sr, Pb, Ni, Co, Cr, Sn, Fe, etc. Alkaline earth metals are particularly preferred because of their solubility in hydrocarbons and potent detergent properties.

In addition to the normal salts of phenolic

compounds, basic salts may be used and can be represented by the formula



wherein the symbols are the same as referred to in the previous formulas. These basic salts may be formed by reacting the aromatic acidic compound with more than the amount of metal oxide or hydroxide necessary to form the normal salt.

Some specific compounds as represented by the above formulas are: barium tertiary octyl phenol sulfide and disulfide, barium di-tertiary amyl phenol sulfide, calcium iso-hexadecyl phenol sulfide, magnesium tertiary amyl phenol sulfide, cobalt tertiary amyl phenol sulfide, barium dodecyl salicylate sulfide, sulfide of the barium salt of the ethyl ester of p-hydroxy dithiobenzoic acid, calcium octyl phenol selenide, etc. The amount of detergent salt used may vary from between about 5 and 15% and preferably is kept below 10%.

In systems wherein substantial amounts of moisture are present, a drying agent may be added which is compatible with the active ingredients of this invention. By tying up most of the free moisture in this manner, the amount which would normally combine with sludge forming materials is diminished, thus alleviating a most aggravating clogging problem.

Drying agents which are particularly suited are the glycol-ether type such as diethylene glycol monomethyl, ethyl, N- and isopropyl ether, diethylene glycol mono-butyl ether, diethylene glycol mono-decyl ether, etc.; also dipropylene glycol mono-ethyl ether, dipropylene glycol mono-isopropyl ether, dipropylene glycol mono-isoamyl ether, diisobutylene glycol-mono isopropyl ether, ethylene-propylene glycol mono-ethyl ether, ethylene - isobutylene glycol mono - isopropyl ether, etc. Instead of the glycol-ethers, various alcohols may be used such as diols having 6 or more carbon atoms in the molecule such as hexylene glycol, decylene glycols, cetylene glycols, etc.; diglycols such as dipropylene glycols, dibutylene glycol, diamylene glycol, ether alcohols and particularly the glycol mono alkyl ethers, e. g. the cellosolves such as ethylene glycol mono ethyl ether, ethylene glycol mono propyl ether, ethylene glycol mono n-butyl ether, ethylene glycol mono iso-butyl ether, ethylene glycol mono tert-butyl ether, ethylene glycol mono hexyl ether, propylene glycol mono ethyl ether, propylene glycol mono isoamyl ether, etc. Also glycerine and the like may be used.

The amount of these drying agent materials, when used, constitutes a substantial portion of the base and generally is around about 50% or more. However, under certain conditions these materials may be omitted from the base.

A general formula of a base concentrate composition of this invention which will henceforth be referred to as Composition A may consist of:

#### COMPOSITION A

|                                                                                    | General Range    | Limited Range   |
|------------------------------------------------------------------------------------|------------------|-----------------|
|                                                                                    | Per Cent<br>2-10 | Per Cent<br>4-8 |
| Salt of a sulfo carboxylic acid ester or a sulfo compound as listed under IB or IC |                  |                 |
| Detergent e. g. Barium salt of an alkyl phenol sulfide                             | 0-10             | 0-8             |
| Drying agent, e. g. diethylene glycol monobutyl ether                              | 0-25             | 0-25            |
| Fuel oil                                                                           | 34-98            | 45-98           |

Specific base compositions may be illustrated by the following examples:

#### COMPOSITION B

|                                 | Per cent |
|---------------------------------|----------|
| Diethyl sodium sulfosuccinate   | 4.0      |
| Hydrocarbon distillate fuel oil | 96.0     |

#### COMPOSITION C

|                                       | Per cent |
|---------------------------------------|----------|
| Diethyl sodium sulfosuccinate         | 8.0      |
| Barium salt of alkyl phenol disulfide | 8.0      |
| Hydrocarbon distillate fuel oil       | 84.0     |

#### COMPOSITION D

|                                       | Per cent |
|---------------------------------------|----------|
| Diethyl sodium sulfosuccinate         | 8.0      |
| Barium salt of alkyl phenol disulfide | 8.0      |
| Diethylene glycol monobutyl ether     | 50.0     |
| Hydrocarbon distillate fuel oil       | 34.0     |

The following table further illustrates suitable anti-clogging base compositions of this invention:

|    | Components <sup>1</sup>            | 1 | 2 | 3 | 4 | 5 | 6 | 7 | 8 | 9 | 10 |
|----|------------------------------------|---|---|---|---|---|---|---|---|---|----|
| 30 | Surface Active Agent:              |   |   |   |   |   |   |   |   |   |    |
|    | Diethyl sodium sulfosuccinate      | x | x | x |   |   |   | x |   | x |    |
|    | Diethyl sodium sulfosuccinate      |   |   |   |   |   |   |   |   |   |    |
|    | Diethyl sodium sulfosuccinate      |   |   |   |   |   |   |   |   |   |    |
| 35 | Detergent:                         |   |   |   |   |   |   |   |   |   |    |
|    | Bar salt of alkyl phenol disulfide |   |   |   | x |   | x |   |   |   | x  |
|    | Ca salt of alkyl phenol disulfide  |   |   |   |   | x |   |   |   | x |    |
| 40 | Ca alkyl salicylate                | x |   |   |   |   |   | x |   |   | x  |
|    | Na alkyl salicylate                |   | x |   |   |   |   |   |   |   |    |
|    | Na petroleum naphthenate           |   |   | x |   |   |   |   |   |   |    |
|    | Ca petroleum naphthenate           |   |   |   |   |   |   | x |   |   |    |
| 45 | Drying Agent:                      |   |   |   |   |   |   |   |   |   |    |
|    | Diethylene glycol monobutyl ether  |   | x | x | x |   |   |   |   |   |    |
|    | Diethylene glycol monoethyl ether  |   |   |   |   |   |   |   |   |   |    |
|    | Ethylene glycol monobutyl ether    |   |   |   |   |   |   |   |   |   |    |
| 50 | Cetylene glycol                    |   |   |   |   |   | x |   | x |   |    |
|    | Dipropylene glycol                 |   |   |   |   |   |   | x |   | x |    |

<sup>1</sup> All of the above compositions are diluted with a hydrocarbon distillate fuel oil in amounts indicated above.

Compositions of this invention are added generally in amounts of 1 pint or less with from about 250 gallons to about 1000 gallons of fuel oil. Thus, for example, on a percentage basis of fuel used, one pint of such compositions described per 250 gallons of fuel would correspond to approximately the following concentration of the active ingredients in the final compositions:

60 Salt of a sulfocarboxylic acid ester or derivatives thereof or compounds as noted under IB and IC, 0.0025% to 0.005%; detergent (salt of an alkyl phenol sulfide), 0 to about 0.0025% or 0.0042%, drying agent (glycol-ether), 0 to 0.0265%.

Compositions B, C and D when added in amounts of approximately 1 pint per 250 gallons of fuel oil correspond to approximately the following concentrations of the active ingredients present in the final composition:

|                               | Per cent by weight |
|-------------------------------|--------------------|
| Diethyl sodium sulfosuccinate | 0.0025             |
| Hydrocarbon fuel oil          | Balance            |

## COMPOSITION C'

## Per cent by weight

|                                     |         |
|-------------------------------------|---------|
| Diethyl sodium sulfosuccinate       | 0.002   |
| Barium salt of alkyl phenol sulfide | 0.0042  |
| Hydrocarbon fuel oil                | Balance |

## COMPOSITION D'

## Per cent by weight

|                                     |         |
|-------------------------------------|---------|
| Diethyl sodium sulfosuccinate       | 0.005   |
| Barium salt of alkyl phenol sulfide | 0.0042  |
| Diethylene glycol monobutyl ether   | 0.0265  |
| Hydrocarbon fuel oil                | Balance |

To inhibit corrosive tendencies of the non-polar organic liquids a minute amount of caustic or aromatic nitrogen compound such as aniline may be added. These compounds act as alkaline reserves and render the fuel, or the hydrocarbon, substantially non-corrosive to copper, brass and other metals.

To illustrate the effectiveness of compositions of this invention as deposit removers, sludge inhibitors and corrosion inhibitors, particularly when the liquid treated has an alkaline reserve, the following tests were made which are self-explanatory.

## Example I

Two 50 cc. samples of a test fuel oil were strained through a 200 mesh screen, in order to remove any extraneous material, and placed in small bottles. To each sample was added 0.15 cc. of distilled water. One sample was retained as a control; the other was doped with a composition containing as active ingredients diethyl sodium sulfosuccinate, barium salt of alkyl phenol disulfide and diethyl glycol monoethyl ether; the total amount of the active ingredients in the doped oil was less than 0.05%. Samples were

30 40

flow through the screen between the doped and undoped oils served as a measure of effectiveness.

| Composition      | Time to flow through screen | Remarks                                                                                             |
|------------------|-----------------------------|-----------------------------------------------------------------------------------------------------|
| Undoped fuel oil | 1,800 seconds               | Screen presented a continuous mass of gelatinized and emulsified sludge which retarded flow of oil. |
| Doped fuel oil   | Less than 25 seconds        | Screen absolutely clean.                                                                            |

## Example II

Approximately 5 gallon samples of undoped and doped fuel oil as in Example I were clouded with steam and circulated for 24 hours through a 100-mesh screen, by means of a conventional oil burner pump. The drop in flow, as measured by a rotameter placed in the stream, indicated the extent to which the screen became clogged during a 24 hour test.

| Composition      | Drop in flow | Remarks                                                            |
|------------------|--------------|--------------------------------------------------------------------|
| Undoped fuel oil | 30%          | Lines, screen, and rotameter heavily coated with sludge and slime. |
| Doped fuel oil   | None         | Apparatus clean.                                                   |

## Example III

Approximately one pint of Composition C was added to about 250 gallons of oil as used in domestic oil burner installations. The strainers in several of the test burners, including the one used in the control test in which the oil was undoped, were thoroughly cleaned at the beginning of the tests, while the strainers in the remaining burners were not cleaned and the test was conducted for about 40 days after which the systems were inspected.

| Test No.                           | 1                                     | 2                        | 3                         |
|------------------------------------|---------------------------------------|--------------------------|---------------------------|
| Inspection at start of test.       |                                       |                          |                           |
| Condition of strainers:            |                                       |                          |                           |
| a. Main fuel line                  | 75% plugged with black sludge.        | 75% coated               | 100% covered.             |
| b. In Nozzle or Magnetic Valve.    | Completely covered with black sludge. | 50% plugged with sludge. | 100% covered with sludge. |
| Time since strainer last cleaned.  | 2 months                              | 1 month                  | 6 months.                 |
| Cleaned at beginning of test?      | Yes                                   | No                       | Yes.                      |
| Amount of oil                      | 500 gallons                           | 500 gallons              | 500 gallons.              |
| Amount of additive (Composition C) | None                                  | 1 quart                  | 1 quart.                  |
| Inspected at end of test:          |                                       |                          |                           |
| Condition of strainers:            |                                       |                          |                           |
| a. Main fuel line                  | 50% plugged                           | Clean                    | Clean.                    |
| b. Nozzle or Magnetic Valve        | 75% covered with black sludge.        | do                       | do.                       |

agitated in a shaking machine for 5 minutes and then put aside for observation.

| Composition      | Observation (Initial)                                                                                                    |
|------------------|--------------------------------------------------------------------------------------------------------------------------|
| Undoped fuel oil | Moisture and particles of emulsion adhered tenaciously to sides of bottle. Black sludge particles dropped to the bottom. |
| Doped fuel oil   | Oil drained evenly and smoothly from side of bottle and solid particles were retained in suspension for a long time.     |

After one hour standing samples were shaken for about 30 seconds and then allowed to flow by gravity through a 200-mesh screen one-fourth inch in diameter. The difference in the rate of

65 70

Fuel tanks were cleaned with acetone and the entire system flushed with kerosene and the tanks charged with 125 gallons of fuel oil to be tested. The oils were steamed with saturated steam for about 1 1/4 minutes. One such oil had an alkaline reserve due to a trace of caustic; the other oil also had an alkaline reserve and was doped with Composition C in amount of less than 0.05%.

The test was conducted for 28 days by circulating the oil through a pump and strainer system and the condition of each specimen as well

## Example IV

as the appearance of the oil and amount of sediment corrosion, etc. observed.

|                                                                   | Per cent |
|-------------------------------------------------------------------|----------|
| Alkali metal salt of an unsubstituted sulfo-carboxylic acid ester | 2-10     |
| Hydrocarbon distillate fuel oil                                   | Balance  |

## WEIGHT LOSS OF TEST SPECIMENS

| Specimens                 | Fuel Oil With Alkaline Reserve (Caustic) | Fuel Oil With Alkaline Reserve (Caustic) and containing less than 0.05% Composition C |
|---------------------------|------------------------------------------|---------------------------------------------------------------------------------------|
| Total Cu Specimens, mg    | 6.9                                      | 1.9                                                                                   |
| Total Brass Specimens, mg | 17.5                                     | 9.9                                                                                   |
| Total All Specimens, mg   | 24.4                                     | 11.8                                                                                  |

## EFFECT OF FUEL OIL DOPED WITH COMPOSITION C ON STRAINERS

| Specimens                                     | Alkaline reserved fuel            | Alkaline reserve oil containing 1 pint of Composition C per 500 gallons oil |
|-----------------------------------------------|-----------------------------------|-----------------------------------------------------------------------------|
| Condition of main line strains.               | 100% covered with brown emulsion. | Lower half slightly stained.                                                |
| Conditions of screen disks in sediment bowls. | 100% covered with brown emulsion. | One screen 10% covered with brown emulsion; other screen clean.             |

To compositions of this invention may be added minor amounts of a foaming inhibitor such as silicon liquids, e. g. dimethyl silicone; fluoro organic compounds, fluoro paraffins, salts of alkyl alkylenephosphates and the like. Compositions of this invention may be used to remove deposits, formed on metal surfaces such as in tubes, evaporators, heat exchangers, distillation and cracking equipment and the like. They are non-corrosive and do not interfere with the functioning of the fluid in which dispersed.

It is understood that while the features of the invention have been described and illustrated in connection with certain specific examples, this invention, however, is not to be limited thereto or otherwise restricted, except by the scope of the appended claims.

We claim as our invention:

1. An anti-clogging concentrate composition suitable for addition to hydrocarbon fuels containing substantial amounts of cracked components and normally susceptible toward clogging comprising:

Per cent

Diocetyl sodium sulfosuccinate 4.0  
Hydrocarbon distillate fuel oil 96.0

2. An anti-clogging concentrate composition suitable for addition to hydrocarbon fuels normally susceptible toward clogging comprising:

Per cent

Diocetyl sodium sulfosuccinate 8  
Barium salt of alkyl phenol disulfide 8  
Hydrocarbon distillate fuel oil Balance

3. An anti-clogging concentrate composition suitable for addition to hydrocarbon fuels containing substantial amounts of cracked components and normally susceptible toward clogging comprising:

Per cent

Diocetyl sodium sulfosuccinate 8  
Barium salt of alkyl phenol disulfide 8  
Diethylene glycol monobutyl ether 50  
Hydrocarbon distillate fuel oil Balance

4. An anti-clogging concentrate composition suitable for addition to hydrocarbon fuels containing substantial amounts of cracked components and normally susceptible toward clogging comprising:

5. An anti-clogging concentrate composition suitable for addition to hydrocarbon distillate fuels containing substantial amounts of cracked components and normally susceptible towards clogging comprising a major amount of a hydrocarbon distillate fuel oil from the group consisting of cracked and mixtures of cracked and straight run fuel oils and a minor amount of from about 2% to about 10% of a metal salt of an unsubstituted sulfoaliphatic dicarboxylic acid ester.

6. An anti-clogging concentrate composition suitable for addition to hydrocarbon distillate fuels containing substantial amounts of cracked components and normally susceptible towards clogging comprising a major amount of a hydrocarbon oil containing a substantial amount of cracked hydrocarbon fractions and a minor amount of from about 2% to about 10% of a salt of an unsubstituted sulfoaliphatic dicarboxylic acid ester.

7. An anti-clogging concentrate composition suitable for addition to hydrocarbon fuel oils containing substantial amounts of cracked components and normally susceptible towards clogging comprising a major amount of a hydrocarbon fuel and a minor amount, sufficient to inhibit clogging, of a salt of an unsubstituted sulfoaliphatic carboxylic acid ester.

8. A non-clogging distillate fuel oil containing entrained moisture normally susceptible to cause clogging due to the presence of cracked components in said fuel oil, said fuel oil rendered non-clogging by incorporating therein about 0.005% diocetyl sodium sulfosuccinate, about 0.0042% barium salt of alkyl phenol disulfide and about 0.0265% diethylene glycol monobutyl ether.

9. A non-clogging distillate fuel oil containing entrained moisture normally susceptible to cause clogging due to the presence of cracked components in said fuel oil, said fuel oil rendered non-clogging by incorporating therein about 0.005% diocetyl sodium sulfosuccinate, about 0.0042% barium salt of alkyl phenol disulfide.

10. A non-clogging distillate fuel oil containing entrained moisture normally susceptible to cause clogging due to the presence of cracked components in said fuel oil, said fuel oil rendered non-clogging by incorporating therein about 0.005% diocetyl sodium sulfosuccinate.

11. A non-clogging distillate fuel oil containing entrained moisture normally susceptible to cause clogging due to the presence of cracked components in said fuel oil, said fuel oil rendered non-clogging by incorporating therein about 0.005% 5 alkali metal salt of an unsubstituted sulfoaliphatic dicarboxylic acid ester.

12. A non-clogging distillate fuel oil containing entrained moisture normally susceptible to cause clogging due to the presence of cracked components in said fuel oil, said fuel oil rendered non-clogging by incorporating therein from about 0.0025 to about 0.005% of a salt of unsubstituted sulfoaliphatic carboxylic acid ester. 10

13. A non-clogging fuel oil normally susceptible 15 to cause clogging due to presence of cracked components in said fuel oil, said fuel oil rendered non-clogging by incorporating therein a salt of an unsubstituted sulfoaliphatic carboxylic acid ester in an amount of about one part of said ester to 20 between 25,000 and 50,000 parts of the fuel oil.

CALMY WIES.

JOHN B. R. CARON.

EVERETT B. GLENDENNING.

#### REFERENCES CITED

The following references are of record in the file of this patent:

#### UNITED STATES PATENTS

| Number    | Name           | Date           |
|-----------|----------------|----------------|
| 2,028,091 | Jaeger         | Jan. 14, 1936  |
| 2,221,839 | Lipkin         | Nov. 19, 1940  |
| 2,296,069 | Talbert et al. | Sept. 15, 1942 |
| 2,316,739 | Cook et al.    | Apr. 13, 1943  |
| 2,362,291 | Winning        | Nov. 7, 1944   |
| 2,369,490 | Proell         | Feb. 13, 1945  |
| 2,456,569 | Smith          | Dec. 14, 1948  |

#### OTHER REFERENCES

"Aerosol," pub. by American Cyanamid & Chem. Corp., 1941, p. 14.